

## UNITED STATES PATENT OFFICE.

EDWARD F. CHANDLER, OF BROOKLYN, NEW YORK.

## FUEL FOR AUTOMOTORS.

No Drawing.

Application filed December 23, 1924. Serial No. 757,731.

This invention relates to liquid fuels for use in internal combustion engines. More particularly this invention pertains to improvements in gasoline or light petroleum distillate for use in automotors.

The primary object of the present invention is to adapt ordinary, commercial gasoline, such as generally offered in the market as motor fuel, for more efficient and satisfactory use in the internal combustion motors of automobiles and other automotors, by improving combustion, increasing operating efficiency, reducing the formation of carbon monoxide and other obnoxious gases in the exhaust, and reducing the deposit of carbon which now attend the operation of gasoline explosion motors.

Other objects will more fully appear during the course of the following description, and the novel features and advantages of the invention will be set forth in the appended claims.

As stated in the premises, this invention does not contemplate the production of a gasoline substitute for use as a fuel in internal combustion engines; but it does aim to produce a fuel for internal combustion engines, the basis of which is gasoline, containing some correcting agents which tend to improve its general performance.

The term "gasoline" does not imply a strictly definite compound having a set chemical composition. While hexane,  $C_6H_{14}$ , may be regarded for the purposes of the present invention as typical of good gasoline, it is well known that wide variations from this standard may be found in the market, owing to varying quantities of a number of different constituents. The term "gasoline" as employed during the course of this description must therefore be understood as meaning the wide variety of light petroleum distillates which are sold and used under this name, and which may vary all the way from a density 0.640 to 0.730, or even more.

In a general way, it may be stated that the feature which characterizes gasoline as compared with kerosene and other heavier distillates, is its volatility, which should at all times be sufficient to permit starting of a motor cold, under all ordinary conditions of temperature.

The enormous development of the automobile in recent years, has made it difficult for the supply of motor fuel to keep up with

the demand. Much study and effort have consequently been devoted to the production of fuels having compounds other than gasoline as a basis, but gasoline still represents the great bulk of the fuel used. However, the great consumption of this product has led to the gradual introduction in the market of lower, or heavier grades, which have manifold increased the problems arising from knocking of the engine and from the formation of carbon deposits on engine parts, as well as from the production of an excessive amount of carbon monoxide in the exhaust.

Much study has therefore also been given to the blending of gasolines from different sources in order to improve the fuel qualities and to cheapen the cost of production, and so as to yield fuels approximating in closest degree to the requirements of an ideal fuel.

In another patent application for "Fuels for internal combustion engines," filed by me November 21, 1924, Serial Number 751,398, I have discussed at length the probable causes of various difficulties in motor operation directly attributable to the nature and composition of the fuel used. From the same it would appear that knocking of an engine where a hydrocarbon of the paraffin series is used as a fuel, is mainly due to a too high percentage of hydrogen in the fuel-air mixture; while on the other hand improper combustion, causing carbon deposits in the engine, as well as the production of carbon monoxide, seems to be mainly due to a deficiency of oxygen in the fuel-air mixtures obtained under carburetor adjustment conditions such as ordinarily used in practice. With certain other fuels, the presence of carbon deposits may be noted even when there is sufficient oxygen available for complete combustion, and in such cases this result may be due to a low ratio of hydrogen in proportion to carbon, and to the resulting low temperature of combustion.

The deficiency of oxygen may be corrected by the addition to the fuel of a compound, such as tetrinitromethane,  $C(NO_2)_4$ , containing sufficient oxygen in excess of that required by its carbon constituent, to improve the combustion conditions of the mixture. This method forms the object of two patent applications previously filed by me, one entitled "Motor fuels," filed October 8, 1924, Serial No. 742,428, and the other en-

titled "Fuels for heat engines," filed October 14, 1924, Serial No. 743,636.

In my other patent application previously referred to, I have explained how the tendency to detonate and the deficiency of oxygen can be corrected at the same time by blending the fuel with substances decreasing the percentage of fuel elements of the fuel-air mixture, at the same time increasing the supply of thermal diluents present; at times increasing also, not only the relative, but also the absolute amount of oxygen in the mixture.

The present invention also refers to fuels having gasoline as a basis, compounded on the same principle; and it represents an improvement over the mixtures advocated in my co-pending application No. 751,398, inasmuch as a certain proportion of alcohol is introduced in the mixture, with beneficial results which I will point out in the course of this description.

The said application refers to a mixture of gasoline, preferably with the addition of a small percentage of kerosene, dimethyl ketone, and water, with or without a small percentage of tetranitromethane or other suitable oxidizing agent.

I have found that by adding alcohol to this mixture, I am enabled to decrease the ratio of dimethyl ketone used, thus to a certain extent reducing the cost of production of the fuel. I am also enabled to decrease the percentage of water, realizing a notable gain in the volatile qualities of the fuel, and at the same time increasing its volumetric efficiency, owing to the high latent heat of vaporization of the alcohol, the usefulness of which is enhanced by the high volatility of the mixture.

The contents of hydrogen and carbon of alcohol are lower than in dimethyl ketone, and therefore a less quantity of combined alcohol and dimethyl ketone is needed to decrease the fuel contents of the fuel-air mixture, than if dimethyl ketone only is used. In this respect methyl alcohol,  $\text{CH}_3\text{OH}$ , is to be preferred to ethyl alcohol,  $\text{C}_2\text{H}_5\text{OH}$ , being also more volatile; but under present conditions ethyl alcohol can be obtained at a somewhat lower price, and considerations of cost will therefore influence the selection of one rather than the other alcohol in various cases.

Alcohol has the tendency to increase the range of fuel-air explosive mixtures, therefore producing a more flexible fuel than ordinary gasoline; it also has the tendency to improve the power output when rich mixtures are used, owing to the increase in mean pressure due to its latent heat of vaporization.

In addition to these advantages, alcohol also has a very low freezing point, and acts as an anti-freezing element in the mixture.

A typical mixture compounded according to the present invention comprises:

|              | Parts by weight. |
|--------------|------------------|
| Gasoline     | 72               |
| Kerosene     | 3 70             |
| Dimethyl ket | 6                |
| Alcohol      | 12               |
| Water        | 7                |

However, if the alcohol used is ethyl instead of methyl alcohol, I prefer to reduce the proportion of water to 6 parts, adding one part of tetranitromethane or other suitable oxidizing agent.

By including both gasoline and kerosene under the denomination of petroleum distillate, various mixtures may be prepared with these ingredients varying between the following proportions:

Petroleum distillate, from 60 to 90 parts; dimethyl ketone, from 1 to 20 parts; alcohol, from 2 to 30 parts; water, from 1 to 10 parts; tetranitromethane, from 0 to 5 parts.

The specific functions of the dimethyl ketone, which may be assisted into the solution by kerosene when needed, are the decrease of the hydrogen contents of the mixture as a whole, reducing the tendency to detonate due to an excessive amount of hydrogen, as well as to an excessive temperature of combustion. At the same time, as a consequence, this ingredient also acts toward reducing the deficiency of oxygen in relation to the fuel elements, both by reducing the percentages of the fuel elements, and by increasing the absolute amount of oxygen in the mixture.

This substance is a liquid having a very good volatility, and will not tend to decrease the volatility of the gasoline. Another advantage of this ingredient is that, being an excellent solvent of carbon, while not contributing towards the prevention of the formation of carbon deposits, it will however cause whatever carbon may be formed to remain in solution, and to be readily expelled with the exhaust.

Owing to this property, the further addition of a combustion supporter, to counterbalance a possible remaining deficiency of oxygen, is therefore optional, in so far as prevention of carbon deposits is concerned.

Water assists the other ingredients in adding its diluting action to reduce the percentage of fuel elements in the fuel-air mixture, and in introducing a powerful thermal diluent; this reduces the tendency to detonate, the temperature of combustion, and heat losses from various causes. The presence of water vapor therefore permits the retention in the mixture of a greater proportion of hydrogen than would otherwise be possible, without detonation. The water vapor has also been found beneficial in exerting a scavenging effect, and in assisting in the prevention of carbon deposits.

The addition of tetranitromethane has for its primary object to furnish some additional oxygen to further improve combustion conditions, incidentally also providing additional nitrogen acting as a thermal diluent; furthermore, owing to its high volatility, it will also tend to improve volatilization of the fuel, which might have been adversely affected by the addition of water. This consideration is not very important in hot climates, but in winter conditions it may become a factor of sufficient importance.

It is obvious that ether, which indirectly also acts as a combustion supporter by decreasing the percentages of the fuel elements, and by increasing the supply of oxygen, and which also has a high vapor tension, may be used instead of tetranitromethane to improve the volatility of the fuel mixture.

20. I claim:

1. A liquid fuel adapted for use in an internal combustion engine, comprising a mixture of gasoline, dimethyl ketone, alcohol, and water.

25. 2. A liquid fuel adapted for use in an internal combustion engine, comprising a mixture of gasoline, kerosene, dimethyl ketone, alcohol, and water.

30. 3. A liquid fuel adapted for use in an internal combustion engine, comprising a mixture of petroleum distillate, dimethyl ketone, alcohol, and water.

35. 4. A liquid fuel adapted for use in an internal combustion engine, comprising a mixture of petroleum distillate, dimethyl ketone, alcohol, water, and a combustion supporter containing oxygen in excess of that required by the combustion of its own combustible elements.

5. A liquid fuel adapted for use in an 40 internal combustion engine, comprising a mixture of petroleum distillate, dimethyl ketone, alcohol, water, and tetranitromethane.

6. A liquid fuel adapted for use in an 45 internal combustion engine, comprising a mixture of petroleum distillate from 60 to 90 parts, dimethyl ketone, from 1 to 20 parts, alcohol, from 2 to 30 parts, and water, from 1 to 10 parts.

7. A liquid fuel adapted for use in an internal combustion engine, comprising a mixture of petroleum distillate from 60 to 90 parts, dimethyl ketone, from 1 to 20 parts, alcohol, from 2 to 30 parts, water, from 1 to 10 parts and a combustion supporter.

8. A liquid fuel adapted for use in an internal combustion engine, comprising a mixture of petroleum distillate from 60 to 90 parts, dimethyl ketone from 1 to 20 parts, 60 alcohol from 2 to 30 parts, water from 1 to 10 parts, and tetranitromethane from 0 to 5 parts.

9. A liquid fuel adapted for use in an internal combustion engine, comprising a 65 mixture of gasoline, 72 parts by weight, kerosene, 3 parts by weight, dimethyl ketone, 6 parts by weight, methyl alcohol, 12 parts by weight, and water, 7 parts by 70 weight.

10. A liquid fuel adapted for use in an internal combustion engine, comprising a mixture of gasoline, 72 parts by weight, kerosene 3 parts by weight, dimethyl ketone 6 parts by weight, ethyl alcohol 12 parts by 75 weight, water 6 parts by weight, and tetranitromethane 1 part by weight.

EDWARD F. CHANDLER.